

1

3,625,693

### THERMALLY DEVELOPABLE DIAZOTYPE COPYING MATERIALS

Takehiko Iwaoka, Tokyo, Japan, assignor to Kabushiki Kaisha Ricoh, Tokyo, Japan  
 No Drawing. Filed Nov. 3, 1967, Ser. No. 680,358  
 Claims priority, application Japan, Nov. 9, 1966,  
 41/73,630  
 Int. Cl. G03c 1/58

U.S. Cl. 96—75

2 Claims

### ABSTRACT OF THE DISCLOSURE

Thermally developable diazotype copying materials comprising a support sheet and a light-sensitive layer supported thereon, said layer containing a light-sensitive diazo compound whose principal component consists of ortho-carboxy benzene diazonium chloride, said layer further containing a coupler, a thermally decomposable alkali generating agent (an agent adapted to produce an alkaline component due to the heat decomposition of said agent) and an acid stabilizer.

### BACKGROUND OF THE INVENTION

#### Field of the invention

The present invention relates to thermally developable diazotype copying materials having a particularly improved shelf life, said copying materials carrying a light-sensitive layer thereon containing a novel light-sensitive diazo compound which is adapted to display its coupling activity only when subjected to a temperature which is 100° C. or higher.

### DESCRIPTION OF THE PRIOR ART

Conventional thermally developable diazotype copying materials employ, as the fundamental components constituting their light-sensitive layers, the following four components which are: a diazo compound, a coupler and an acid stabilizer, all of which have been used in the so-called dry development copying materials as well as in the wet development copying materials, and also a thermally decomposable alkali generating agent. However, the thermally decomposable alkali generating agent which is contained as a coupling accelerator in the copying materials of the prior art had a disadvantage that it became gradually decomposed during the storage of the copying materials, causing the acid stabilizer to be neutralized, resulting in an elevation of the pH value of the light-sensitive layer and accordingly causing a premature coupling between the diazo compound and the coupler to take place. Thus, the storage of the development type copying materials for an extended period of time results not only in a loss of clear images on the prints obtained, but also gave rise to instances where the copying materials were no longer usable because of the occurrence of the so-called fog effect.

### SUMMARY OF THE INVENTION

The present invention is concerned with thermally developable diazo-type copying materials which are featured by the inclusion, in the light-sensitive layer of the following fundamental component which consists of an ortho-carboxy diazonium compound which will be described later.

It is the object of the present invention to eliminate the shortcomings of the copying materials of the prior art and to provide a copying material which is of an improved shelf life and which permits the user to obtain a clear image of print, by conducting the development at

2

an elevated temperature (under heat development conditions; a temperature ranging from 100° C. to 200° C., and a development time ranging from 2 to 10 seconds).

More specifically, it is the primary object of the present invention to provide a thermally developable diazotype copying material having a markedly improved shelf life.

Another object of the present invention is to provide a light-sensitive diazonium compound which is outstandingly suitable for use in thermally developable diazotype copying materials.

The diazo compounds which are used in the present invention can be classified into the following four groups:

(a) Compounds represented by the general formula:



wherein: R<sub>1</sub> and R<sub>2</sub> are selected from the group consisting of hydrogen; aryl radicals; alkyl radicals having 1 to 4 carbon atoms; and hydroxy alkyl radicals having 1 to 4 carbon atoms, and X is selected from the group consisting of hydrogen, alkyl radicals having 1 to 4 carbon atoms and alkoxy radicals having 1 to 4 carbon atoms.

(b) Compounds represented by the general formula:



wherein: Y is selected from the group consisting of —CO—NH—, —S—, and —NH—, and X is selected from the group consisting of hydrogen, alkyl radicals having 1 to 4 carbon atoms and alkoxy radicals having 1 to 4 carbon atoms.

(c) Compounds represented by the general formula:



wherein:

Y' is selected from the group consisting of a morpholino radical, a pyrrolidinyl radical and a piperazinyl radical, and

X' is selected from the group consisting of hydrogen, alkyl radicals having 1 to 4 carbon atoms and alkoxy radicals having 1 to 4 carbon atoms.

(d) Compounds represented by the general formula:



wherein: Z is selected from the group consisting of alkoxy radicals having 1 to 4 carbon atoms and X' is selected from the group consisting of halogen, alkyl radicals having 1 to 4 carbon atoms and alkoxy radicals having 1 to 4 carbon atoms.

These ortho-carboxy diazo compounds represented by the foregoing general formulas (a) through (d), or more specifically, the compounds whose principal component consists of ortho-carboxy benzene diazonium chloride are markedly stable even in an alkaline atmosphere and do not give rise to coupling even in the presence of couplers. However, these compounds gain coupling activity only when subjected to an elevated temperature, and at such time they easily react with the couplers which are in contact with these compounds. In other words, those ortho-carboxy diazo compounds enumerated above do not

possess coupling activity at normal temperature, but they gain coupling ability for the first time when they are heated to 100° C. or higher. Such nature of these particular compounds has not been elucidated yet. It is presumed, however, that the diazo radical and carboxyl radical contained in said diazo compounds form a secondary bonding at normal temperature, having a structure which is quite stable in an alkaline atmosphere and with no coupling activity of their own. It is considered further that, by heating the compounds to 100° C. or higher, the aforesaid secondary-bonding between these radicals is destroyed, converting the compounds into such diazo compounds as have coupling activity, so that in case the heated compounds containing a coupler is placed in an alkaline atmosphere, the compounds instantaneously couple with the coupler to form a dyestuff. In the present invention, these ortho-carboxy diazo compounds are used in the form of borofluoride or metal double salts such as zinc chloride and cadmium chloride.

Description will next be directed to examples of preparation of these diazo compounds.

(1) P-dimethylamino-O-carboxy-benzene diazonium chloride-cadmium chloride double salt

P-dimethylamino-O-carboxyl-aniline was dissolved in a solution consisting of 50 cc. of water and 16 gr. of 12 N hydrochloric acid. To this mixed solution which was cooled to a temperature ranging from 0° C. to 5° C. was added 3 gr. of sodium nitrite (NaNO<sub>2</sub>). The reaction was completed at the end of about one hour of continuous stirring at said temperature. After filtering the resulting solution, cadmium chloride was gradually introduced into the filtered solution, with the result that a yellow precipitate was formed. After filtering this precipitate, it was recrystallized with water. As the result, the captioned diazo compound having a melting point of 174° C. was obtained.

(2) P-diethyl-m-ethoxy-O-carboxy-benzene diazonium chloride-cadmium chloride double salt

In exactly the same manner as in (1), the captioned diazo compound was formed from P-diethyl-m-ethoxy-O-carboxy-aniline.

(3) P-benzoylamino-m-ethoxy-O-carboxy-benzene diazonium borofluoride

30 gr. of P-benzoylamino-m-ethoxy-O-carboxy-aniline and 9 gr. of sodium nitrite were dissolved in 50 cc. of water. The resulting solution which was cooled to 0° C.-3° C. was gradually added to 50 cc. of an aqueous solution containing 20 cc. of undiluted hydrochloric acid (12 N) which was held at 0° C.-3° C. while stirring the mixture. After the completion of this admixture, stirring was continued for 30 minutes, followed by the addition of sodium fluoroborate (NaF<sub>4</sub>B). As a result, a precipitate was formed. After filtering the precipitate, the latter was recrystallized with water. Thus, yellow crystals of the captioned diazo compound having a melting point of 178° C. was obtained.

(4) P-morpholino-O-carboxy-benzene diazonium chloride-cadmium chloride double salt

23 gr. of P-morpholino-O-carboxy-aniline and 25 cc. of undiluted hydrochloric acid (12 N) were dissolved and dispersed in 100 cc. of water. While stirring, the resulting solution held at 0° C.-3° C. and 9.0 gr. of sodium nitrite was gradually added thereto. After completion of the admixture, stirring was continued for about one hour, at the end of which diazotization was completed. Upon the addition of cadmium chloride to the resulting solution, there was formed a yellow precipitate. The filtered precipitate was subjected to re-crystallization which was repeated twice. As a result, beautiful yellow crystals of the captioned diazo compound was obtained.

The couplers which are used in the present invention include known couplers which have been used in the con-

ventional dry development copying materials and wet development copying materials. They include, for example, 2,3-dihydroxy-naphthalene-6-sodium sulfonate, 1-hydroxy-naphthalene-4-sodium sulphate, R-acid, naphthol AS, 2,3-dihydroxy naphthalene, 2,7-dihydroxy naphthalene 3,6-disodium sulfonate and NW-acid.

Similarly, as the acid stabilizers there can be employed those which have been used in the conventional dry development copying materials and wet development copying materials. They include, for example, tartaric acid, citric acid, oxalic acid, malonic acid, maleic acid, sulphuric acid and phosphoric acid.

Thermally decomposable alkali generating agents which are used in the present invention are such that they are neutral at normal temperature, but they produce alkaline substances when heated to 100° C. or higher.

The thermally decomposable alkali generating agents include:

- 20 (a) Urea and its derivatives: urea, phenyl-urea, methyl-urea, ethyl-urea, hydroxyethyl-urea, acetyl-urea, 1,3-dimethyl-urea.
- (b) Thiourea and its derivatives: thiourea, thioacetamide, guanyl-o-methyl-isothiourea, methyl-isothiourea.
- 25 (c) Guanidine and its derivatives: guanidine, amino-guanidine, guanyl-urea, biguanidine, methyl-biguanidine, o-methyl-guanyl urea, cyanoguanidine.
- (d) Acid amide compounds: acetamide, acryl-amide, propionamide, butylamide, malonamide, salicylamide.
- 30 (e) Salts which were produced with trichloroacetic acid and basic component: sodium trichloroacetate, potassium trichloroacetate, ammonium trichloroacetate, calcium trichloroacetate, dimethylamine-trichloroacetate, diethylamine - trichloroacetate, monomethylamine-trichloroacetate, triethanolamine-trichloroacetate, guanidine-trichloroacetate, aminoguanidine-trichloroacetate.
- 35

These thermally decomposable alkali generating agents are added either independently or in combination of two or more of them to the light-sensitive layer.

The thermally developable diazotype copying materials of the present invention are manufactured by first preparing a solution adapted for forming a light-sensitive layer by mixing, with appropriate ratio by weight, one of the aforesaid diazo compounds, one of the aforesaid couplers, one of the aforesaid acid stabilizers and one or combination of two or more of the aforesaid thermally decomposable alkali generating agents, thereafter applying this solution uniformly onto the upper face of the supporting sheet in an amount in the range of from 40 to 60 gr./m.<sup>2</sup> and then drying the coated sheet. The supporting sheets are not restricted to paper alone, but they can be selected, as desired, from various sheet materials such as precoated paper cloths and plastic foils.

As has been described above, the thermally developable diazotype copying materials of the present invention carry thereon a light-sensitive layer containing a novel diazo compound which does not display its coupling ability unless heated to 100° C. or higher. Therefore, there takes place absolutely no premature coupling phenomenon between the diazo compound and the coupler even after the copying materials have been stored for an extended period of time. Besides, by the use of the copying materials of the present invention in taking copies of originals, there are formed very clear images on the prints by subjecting the exposed sheets to heat development at a temperature ranging from 100° C. to 200° C. for two to ten seconds. Moreover, when the exposed copying materials of the present invention are developed in ammonia gas or an alkaline developing solution in a manner similar to that for the conventional dry or wet development copying materials, there takes place hardly any coupling phenomenon between the diazo compounds and the couplers, and accordingly, no color development is effected.

## DESCRIPTION OF THE PREFERRED EMBODIMENTS

## Example 1

|                                                                                    |       |       |
|------------------------------------------------------------------------------------|-------|-------|
| P-dimethylamino-ortho-carboxy-benzene diazonium chloride·zinc chloride double salt | ----- | Gr. 5 |
| 2,3-dihydroxy-naphthalene-6-sodium sulphonate                                      | ----- | 1.0   |
| Tartaric acid                                                                      | ----- | 2.0   |
| Urea                                                                               | ----- | 1.0   |
| Water                                                                              | ----- | 20.0  |
|                                                                                    |       | 100.0 |

A solution consisting of the above composition was uniformly applied onto the face of a supporting sheet to an extent of 50 gr./m.<sup>2</sup>, followed by drying. As the result, a thermally developable diazotype copying material having a markedly improved shelf life was obtained. An original was placed on this copying material and the assembly was exposed to ultraviolet ray irradiation and then the exposed sheet was subjected to heat development at 150°C. for five seconds, with the result that a very clear blue color image was obtained.

For comparison, a thermally developable copying material was prepared by substituting said P-dimethylamino-O-carboxy benzene diazonium chloride·zinc chloride double salt with P-dimethylamino-benzene diazonium chloride. The obtained copying material had a too poor shelf life to be suitable for practical use. For example, the developed copying material of the present invention was compared with the control copying material as to the fog density resulting from subjecting these two to five day forced aging at 50°C. and at a relative humidity of 20%.

The result was as follows:

|                                  |             |
|----------------------------------|-------------|
|                                  | Fog density |
| Product of the present invention | 0.12        |
| Control                          | 0.70        |

## Example 2

|                                                                                   |       |        |
|-----------------------------------------------------------------------------------|-------|--------|
| P-benzoylamino - O - carboxy-benzene diazonium chloride·zinc chloride double salt | ----- | Gr. 40 |
| NW-acid                                                                           | ----- | 1.0    |
| Sodium trichloroacetate                                                           | ----- | 2.5    |
| Urea                                                                              | ----- | 3.0    |
| Thiourea                                                                          | ----- | 5.0    |
| Pyrophosphate                                                                     | ----- | 5.0    |
| Water                                                                             | ----- | 1.5    |
|                                                                                   |       | 45     |
|                                                                                   |       | 100.0  |

A solution having the above composition was applied onto the face of a supporting sheet and was dried in a manner similar to that described in Example 1, and thus a copying material having a markedly improved shelf life was obtained. The developed image on this print was bluish-violet in color, making a good contrast to the background.

For comparison, a thermally developable copying material was prepared by substituting said P-benzoylamino-O-carboxy-benzene diazonium chloride·zinc chloride double salt with P-benzoylamino-benzene diazonium chloride·zinc chloride double salt. The obtained copying material had a too poor shelf life to be applicable for practical use.

## Example 3

|                                                                                 |       |        |
|---------------------------------------------------------------------------------|-------|--------|
| P-morpholino-m-ethoxy-O-benzene diazonium chloride·cadmium chloride double salt | ----- | Gr. 65 |
| 2,3-dihydroxy-naphthalene-6-sodium sulphonate                                   | ----- | 1.0    |
| Sodium trichloroacetate                                                         | ----- | 2.5    |
| Urea                                                                            | ----- | 3.0    |
| Pyrophosphate                                                                   | ----- | 10.0   |
| Water                                                                           | ----- | 1.5    |
|                                                                                 |       | 70     |
|                                                                                 |       | 100.0  |

A solution having the above composition was applied onto the face of a supporting sheet and dried in a manner similar to that described in Example 1, and a copying material having a markedly improved shelf life was

obtained. The developed image on this copying material was sky-blue which was very clear.

For comparison, thermally developable copying materials were prepared by substituting said P-morpholino-m-ethoxy-O-carboxy benzene diazonium chloride·cadmium chloride double salt with P-morpholino-m-ethoxy-benzene diazonium chloride or with P-morpholino-2,5-diethoxy-benzene diazonium chloride·cadmium chloride double salt. The obtained copying materials developed premature coupling at normal temperature, resulting in an extremely poor shelf life this making it not suitable for practical use.

Although particular preferred embodiments of the invention have been disclosed for illustrative purposes, it will be recognized that variations or modifications of such disclosure, which come within the scope of the appended claims, are fully contemplated.

The embodiments of the invention in which an exclusive property or privilege is claimed are defined as follows;

1. In a thermally developable diazotype copying material having on one surface of a supporting sheet a light-sensitive layer comprising a light-sensitive diazo compound, a coupler, a thermally decomposable alkali generating agent and an acid stabilizer, the improvement wherein said light-sensitive diazo compound consists of at least one double salt of a metal halide with a compound selected from the group consisting of the compounds of the following Formulas *a* through *c*,

(a)



wherein:

*Y* is selected from the group consisting of —CO—NH—, —S—, and —NH, and *X* is selected from the group consisting of hydrogen, alkyl radicals having 1 to 4 carbon atoms and alkoxy radicals having 1 to 4 carbon atoms;

(b)



wherein:

*Y'* is selected from the group consisting of a morpholino radical, a pyrrolidinyl radical and a piperazinyl radical, and

*X'* is selected from the group consisting of hydrogen, alkyl radicals having 1 to 4 carbon atoms and alkoxy radicals having 1 to 4 carbon atoms; and

(c)



wherein:

*Z* is selected from the group consisting of alkoxy radicals having 1 to 4 carbon atoms and *X''* is selected from the group consisting of halogen, alkyl radicals having 1 to 4 carbon atoms and alkoxy radicals having 1 to 4 carbon atoms,

and said coupler is a member selected from the group consisting of 2,3 - dihydroxy-naphthalene-6-sodium sulfonate, 1-hydroxy-naphthalene-4-sodium sulphate, R-acid, naphthol AS, 2,3 - dihydroxy-naphthalene, 2,7 - dihydroxy-naphthalene-3,6-disodium sulfonate and NW-acid, the amounts of the diazo compound and the coupler

being effective to react at temperatures in excess of about 100° C. to form a visible image and the diazo compound and the coupler being substantially non-reactive in the presence of ammonia gas or an alkaline developing solution.

2. Improvement in a thermally developable diazotype copying material according to claim 1, wherein said thermally decomposable alkali generating agent consists of at least one compound selected from the group consisting of urea, phenyl-urea, methyl-urea, ethyl-urea, hydroxy-ethyl-urea, acetyl-urea, 1,3-dimethyl-urea, thiourea, thioacetamide, guanyl-O-methyl-isothio-urea, methyl-isothiourea, guanidine, amino-guanidine, guanyl-urea, biguanidine, methyl-biguanidine, O-methyl-guanyl-urea, cyano-guanidine, acetamide, acrylamide, propionamide, butylamide, malonamide, salicylamide, sodium trichloroacetate, potassium trichloroacetate, ammonium trichloroacetate, calcium trichloroacetate, dimethylamino-trichloroacetate, diethylamine-trichloroacetate, monomethyl-

amine-trichloroacetate, triethanolamine-trichloroacetate, guanidine-trichloroacetate and amino-guanidine-trichloroacetate.

#### References Cited

| UNITED STATES PATENTS |         |           |         |
|-----------------------|---------|-----------|---------|
| 1,807,761             | 6/1931  | Spongerts | 96—91   |
| 2,066,918             | 1/1937  | Vonposer  | 96—91 X |
| 2,532,126             | 11/1950 | Slifkin   | 96—91   |
| 3,360,371             | 12/1967 | Munder    | 96—91   |
| 3,434,838             | 3/1969  | Munder    | 96—49 X |

WILLIAM D. MARTIN, Primary Examiner

W. R. TRENOR, Assistant Examiner

U.S. Cl. X.R.

96—47, 91; 260—141